

## UNITED STATES PATENT OFFICE

2,164,798

HYDROLYTIC DECOMPOSITION PRODUCT  
OF THE EPIDERMIS OF HOGS, ETC.

Charles H. Campbell, Kent, Ohio

No Drawing. Original application May 3, 1938,  
Serial No. 211,044. Divided and this applica-  
tion November 15, 1938, Serial No. 240,454

2 Claims. (Cl. 260—112)

This invention relates to products obtained by the hydrolytic decomposition of the epidermis of hogs and such foreign matter as may be present after removal and separation of the hair or bristles from said epidermis. This application is 5 a division of my application Ser. No. 211,044, filed May 3, 1938.

The derivatives or cleavage products resulting 10 from my invention provide an excellent reinforcing agent or filler for rubber possessing no properties harmful to rubber over a long period of time. More particularly this reinforcing agent or filler is capable of making the rubber soft, tacky and dead in character before vulcanizing 15 though resilient, elastic and tough with an excellent grain when vulcanized.

The derivatives or cleavage products produced 20 in accordance with my invention are those obtained by the hydrolytic decomposition of the epidermis of hogs to the point of obtaining soluble and diffusible cleavage products but preferably short of such hydrolytic decomposition as will form amino-acids, though some may be present, and preferably also those soluble and diffusible 25 cleavage products obtained by the hydrolytic decomposition of the epidermis of hogs through the influence of heat and pressure by steam.

In this country, the slaughtering and subsequent treatment of hogs is usually carried out 30 in a manner that permits recovery of the epidermis, and prior to my invention the epidermis was disposed of as waste which had no known value of any consequence. After killing, the hogs are subjected to a scalding treatment which 35 loosens the epidermis from the under skin and then they are scraped. This scraping removes the epidermis and dehairs the animals, providing a mixture of epidermis, hair and bristles which is cleansed or washed with a suitable agent 40 and the hair and bristles separated from the epidermis, the latter being thrown away as waste. The foregoing treatment of hogs is well understood in the art.

The epidermis remaining after the separation 45 of hair and bristles, after being subjected to further treatment that will be referred to, is the material I use to produce my product. While there may be some impurities in this material, such as very short hairs which are unavoidably 50 retained, a little blood albumen, and possibly a small amount of salts which are usually found in the epidermis of any animal, the material constitutes largely the epidermis and is to be so considered herein.

55 I take the recovered epidermis and place it in

a closed digester to hydrolyze and decompose it. Hydrolytic decomposition is effected by admitting steam to the digester and in some instances a small amount of caustic soda may be added. Steam admitted at 100 lbs. pressure for approximately two hours has been found to be ample in connection with the epidermis obtained from young animals. With the older epidermis, however, it is desirable to carry on the digesting process for a longer period of time as for example even 10 up to six hours. The process can be hastened, however, by increasing the steam pressure or superheating the steam. The difficulty with the higher steam pressures, however, especially when epidermis of a miscellaneous type is being treated 15 in large quantities at one time, such as 15,000 to 20,000 pounds or more, is that the higher steam pressures when long continued are apt to have a too drastic action on the epidermis and produce an undue proportion of the amino-acids. Accordingly 20 it is desirable to raise the steam pressure gradually and to remove the soluble cleavage products at intervals rather than make one long digestion to prevent the first fraction of cleavage products formed, from hydrolyzing through into 25 the amino-acid group although at times some may be present. Thus steam might first be admitted to the digester at about 60 pounds pressure for about two hours, the steam then shut off, pressure on the digester relieved and the soluble products thus far formed removed. Steam might then be admitted at 80 pounds pressure for a further period of two hours, the steam then 30 shut off, the pressure relieved and the soluble products again removed. Steam may then well 35 be admitted to the digester at 100 pounds pressure for a period of at least two hours depending upon the condition of the mass within the digester. The resulting material is a flowable liquid, usually of a dark color, in which the epidermis 40 has been fully dissolved.

At the expiration of the hydrolyzing process the liquid material is passed to a suitable dryer wherein all except about 2% to 3% of the moisture content is preferably removed. Any commonly accepted drying process may be used and I prefer to use either an open pan or a stick roll in drying. This gives us a dried, solid material which is next ground up into a fine powder, which should be immediately bagged in moisture- 45 proof bags to prevent caking.

The epidermis derivatives thus obtained constitute a very satisfactory reinforcing agent or filler for rubber which is mixed or compounded preferably in its powdered form with the rubber, 55

before vulcanizing in the ordinary manner. In compounding reclaims the powder is preferably added after the rubber leaves the dryer, the rubber usually having enough moisture content to permit dispersion of the powder through the rubber. With natural rubber it is desirable, though not necessarily essential, to make up a master batch with my powder in it and then use the desired percentage of the master batch with additional rubber.

The epidermis is an albuminous protein distinctly different in character and makeup from keratin, collagen or elastin, which are also animal proteins. With the latter animal proteins it usually requires from 3% to 6% thereof by weight added to rubber in order to produce the desired result, whereas, with the present material as little as 2% by weight can be satisfactorily used, producing a result which, according to tests made, is as high as 20% better than has heretofore been possible with other materials, this increase being noticeable in both the compounded product and the finished product.

Among the reasons why rubber compounded with epidermis is more satisfactory is that epidermis does not appear to be detrimentally af-

fected by the high temperatures used in treating rubber. The finished rubber product is resilient and pliable, is capable of a very large number of flexing actions without cracking, is tough, and is not subject to the deterioration that sometimes takes place when other animal products are compounded with rubber.

It will be apparent that modifications of the invention may be resorted to without departing from the spirit thereof or from the scope of the 10 subjoined claims.

What is claimed is:

1. A new product of manufacture comprising the hydrolytic decomposition products of the epidermis of hogs and such foreign matter as may be present after removal and separation of the hair or bristles from said epidermis, and which products are substantially short of amino-acids.
2. A new product of manufacture comprising soluble and diffusible hydrolytic decomposition products of the epidermis of hogs and such foreign matter as may be present after removal and separation of the hair or bristles from said epidermis, and which products are substantially short of amino-acids.

CHARLES H. CAMPBELL.

25

5

10

15

20

25